

## UNITED STATES PATENT OFFICE

2,351,791

## ALLOY

Jacob Trantin, Jr., Youngstown, Ohio

No Drawing. Application January 5, 1942,  
Serial No. 425,665

2 Claims. (Cl. 75—125)

This invention relates to ferrous alloys in the steel range which may be readily cast, and which have high wear-resistance and freedom from scale pick-up.

It is the general object of my invention to provide an improved alloy which may be directly and readily cast into members for guiding, forming, or working hot metal or other materials and characterized by toughness, wear-resistance, corrosion-resistance, and lack of susceptibility of metal deposit thereon.

Another object of my invention is the provision of an improved ferrous alloy including chromium, copper, cobalt, silicon, manganese, and molybdenum.

Another object of my invention is to provide improved articles for piercing, guiding, forming or working hot metal or the like which articles have a greatly prolonged life over that of known members now in use for this purpose, and characterized by lack of susceptibility to scale pick-up and by corrosion and wear-resistance.

The foregoing and other objects of my invention are achieved by the provision of an alloy including .20 to 2.00 per cent carbon, about 5.00 to about 30.00 per cent chromium, 5.00 to about 15.00 per cent copper, 1.00 to about 10.00 per cent cobalt, .10 to about 3.00 per cent molybdenum, .30 to 1.50 per cent silicon, .05 to 1.75 per cent manganese, up to 1.50 per cent vanadium, and the remainder substantially all iron.

I may keep the limits of my improved alloy as follows: carbon .40 to .99 per cent, chromium 11.0 to 18.0 per cent, copper 6.0 to 9.0 per cent, cobalt 2.5 to 4.5 per cent, molybdenum .5 to 1.5 per cent, silicon .3 to 1.5 per cent, vanadium .1 to .50 per cent, manganese .4 to .9 per cent, and the remainder substantially all iron.

One typical heat of the alloy of my invention which possesses the improved characteristics above set forth comprises the following composition: carbon about .8 per cent, chromium about 15.0 per cent, copper about 7.5 per cent, cobalt about 4.0 per cent, molybdenum about .75 per cent, silicon about .80 per cent, vanadium about .25 per cent, manganese about .60 per cent, and the remainder substantially all iron.

In the several examples given, traces of other materials are not objectionable, nor are the usual percentages of sulphur and phosphorus present in open hearth or Bessemer commercial steels.

The cobalt and molybdenum present in my alloy are believed to bear such a relation to each

other that when the cobalt content is increased the molybdenum content may be reduced, and, when the molybdenum content is increased the cobalt content may be reduced. In any event, it is advisable to keep the combined molybdenum and cobalt contents in the alloy between about 4.00 and about 10.00 per cent of the total alloying ingredients.

Further, the manganese and chromium present in the alloy bear a relation to each other so that if the manganese content is increased above the limits hereinabove noted then the chromium content can be reduced by an amount substantially equal to the increase in the manganese content.

15 In any event, the combined amounts of chromium and manganese present in the alloy should be within the limits of between about 5.00 and about 30.00 per cent. I have found, also, that instead of using vanadium in the amounts indicated that 20 I may employ aluminum in similar amounts to achieve substantially the same results in the alloy.

From the foregoing it will be recognized that the objects of my invention have been achieved and that I have provided a castable ferrous alloy, particularly adapted to act as a guiding or forming member for hot metal and the like, and characterized by wear-resistance, corrosion-resistance and long life without the deposition of scale thereon.

30 Although in accordance with the patent statutes, I have particularly described my invention, it will be understood that I am not to be limited thereto or thereby, but that the scope of my invention is defined in the appended claims.

35 I claim:

1. A ferrous alloy comprising about .8 per cent carbon, about 15.00 per cent chromium, about 7.50 per cent copper, about 4.0 per cent cobalt, about .75 per cent molybdenum, about .80 per cent silicon, about .25 per cent vanadium, about .60 per cent manganese, and the remainder substantially all iron, said alloy being characterized by wear-resistance, corrosion resistance, and freedom from hot metal scale pick-up.

45 2. A ferrous alloy having an analysis including: carbon .40 to .99 per cent; chromium 11.00 to 18.00 per cent; copper 6.00 to 9.00 per cent; cobalt 2.5 to 4.5 per cent; molybdenum .5 to 1.5 per cent; silicon .3 to 1.5 per cent, vanadium .1 to .50 per cent; manganese .4 to .9 per cent; and the remainder substantially all iron, said alloy being characterized by wear-resistance.

JACOB TRANTIN, JR.